

Patented May 16, 1939

2,158,651

# UNITED STATES PATENT OFFICE

2,158,651

## STEEL

Frederick M. Becket, New York, and Russell Franks, Niagara Falls, N. Y., assignors to Electro Metallurgical Company, a corporation of West Virginia

No Drawing. Application June 24, 1936,  
Serial No. 87,006

7 Claims. (Cl. 75—123)

This invention relates to steels, and provides new and improved steels characterized by novel and commercially valuable properties.

We have discovered that the addition of columbium in amounts between 0.02% and 1% to so-called "plain carbon" and certain "low alloyed" steels effects a marked and surprising improvement in the properties of such steels. One important effect of the columbium addition is to refine the grain-size of the steel, and this grain refinement is retained and maintained even at elevated temperatures up to and somewhat above the critical range. Another effect, which is doubtless at least in part a result of the grain refinement, is the improvement of the tensile strength of many of the steels. Further, the impact strength is increased, and this improvement is marked even at subzero temperatures. There is also an increase in the resistance of the steels to rusting and hot oxidation. The deep-drawing and cold-rolling characteristics of the steels are improved. The hardenability of the steels by heat treatment is somewhat decreased, and there is less distortion of the steel when it is rapidly cooled from elevated temperatures. The ratio of yield point to maximum stress is increased, the increase depending upon the columbium and carbon contents of the steels: the increase is greater in the steels having the lower carbon and columbium contents.

30 Steels included in our invention are:

A. Plain carbon steels containing carbon in amounts not exceeding 1% and preferably not exceeding 0.6%, silicon in amounts up to 1%, manganese in amounts up to 2%, and suitable amounts of columbium, the remainder iron.

B. Chromium steels containing carbon in amounts not exceeding 0.6% and preferably not over 0.4%, 0.25% to less than 2% chromium, silicon in amounts up to 1%, manganese in amounts up to 2%, suitable amounts of columbium, and the remainder iron.

C. Chromium-nickel steels containing, in addition to the ingredients of the chromium steels, 0.05% to 5% nickel. The manganese preferably does not exceed 1%.

D. Molybdenum steels containing carbon in amounts up to 0.6% and preferably not over 0.4%, 0.05% to 1% molybdenum, manganese in amounts up to 2%, silicon in amounts up to 1%, suitable amounts of columbium, and the remainder iron.

E. Molybdenum-nickel steels containing, in addition to the ingredients of the molybdenum steels, 0.05% to 5% nickel. The manganese in these steels preferably does not exceed 1%.

F. Chromium-molybdenum steels containing carbon in amounts up to 0.6% and preferably not

over 0.4%, 0.25% to 2% chromium, 0.05% to 1% molybdenum, silicon in amounts up to 1%, manganese in amounts up to 2%, suitable amounts of columbium, and the remainder iron.

Suitable amounts of columbium to be added to these steels according to the present invention are from 0.02% to 1%. Usually, it will not be necessary or desirable to exceed 0.5% columbium, and the most useful range is within the limits 0.05% to 0.25%. In general, the greater amounts of columbium should ordinarily be used in the steels containing the greater amounts of carbon, within the ranges specified above.

One of the most valuable properties of the columbium containing steels of the invention is that of retaining its normally fine grained structure at elevated temperatures, which property is attained without detrimentally affecting other important physical properties. The expedients heretofore customarily employed to refine the grain size of carbon and low-alloyed steels have, in most cases, either detrimentally affected the toughness of the steels, or failed to prevent coarsening of the grain size at elevated temperatures, during fabrication for instance, or both. The coarsening of the grain is considerably aggravated in a case carburizing process, and in such a process the addition of columbium to the steel is especially advantageous, as illustrated by the data in Table I which gives the experimentally determined grain number (A. S. T. M. Specification E 19-33) of the cases of a series of steels after carburizing for eight hours at each of three different temperatures. In each case, the grain size of the core was smaller than that of the case.

Table I

| % C  | Composition of steel (remainder iron) |      |       |              |        | Grain No. of case after carburizing 8 hours— |            |             | 40 |
|------|---------------------------------------|------|-------|--------------|--------|----------------------------------------------|------------|-------------|----|
|      | % Mn                                  | % Si | % Cb  | Other metals |        | At 925° C.                                   | At 975° C. | At 1025° C. |    |
| 0.16 | 0.46                                  | 0.29 | None  | None         | 3 to 5 | 3 to 5                                       | 1 to 4     |             | 45 |
| 0.15 | 0.45                                  | 0.27 | 0.017 | None         | 3 to 8 | 3 to 8                                       | 2 to 8     |             |    |
| 0.17 | 0.48                                  | 0.26 | 0.46  | None         | 7 to 8 | 5 to 8                                       | 5 to 8     |             |    |
| 0.41 | 0.77                                  | 0.27 | None  | None         | 2 to 4 | 1 to 4                                       | 1 to 4     |             | 50 |
| 0.33 | 0.80                                  | 0.27 | 0.06  | None         | 5 to 7 | 4 to 7                                       | 5 to 7     |             |    |
| 0.43 | 0.74                                  | 0.22 | 0.36  | None         | 6 to 8 | 6 to 8                                       | 5 to 8     |             |    |
| 0.77 | 0.75                                  | 0.22 | None  | None         | 1 to 3 | 1 to 3                                       | 1 to 3     |             | 55 |
| 0.94 | 0.75                                  | 0.25 | 0.04  | None         | 5 to 7 | 4 to 6                                       | 4 to 6     |             |    |
| 0.93 | 0.73                                  | 0.24 | 0.18  | None         | 6 to 7 | 6 to 7                                       | 5 to 8     |             |    |
| 0.97 | 0.72                                  | 0.19 | 0.41  | None         | 5 to 8 | 5 to 8                                       | 5 to 8     |             |    |
|      |                                       |      |       | % Ni         |        |                                              |            |             |    |
| 0.15 | 1.50                                  | 0.16 | None  | None         | 1 to 3 | 1 to 3                                       | 1 to 3     |             |    |
| 0.17 | 1.61                                  | 0.33 | 0.12  | None         | 5 to 8 | 5 to 8                                       | 5 to 8     |             |    |
| 0.52 | 1.68                                  | 0.36 | 0.11  | None         | 5 to 8 | 5 to 8                                       | 4 to 8     |             |    |
|      |                                       |      |       |              |        |                                              |            |             |    |
| 0.16 | 0.36                                  | 0.16 | None  | 3.49         | 2 to 6 | 2 to 6                                       | 2 to 7     |             |    |
| 0.37 | 0.40                                  | 0.17 | None  | 3.52         | 5 to 9 | 3 to 8                                       | 2 to 7     |             |    |
| 0.17 | 0.47                                  | 0.31 | 0.10  | 3.45         | 6 to 9 | 6 to 9                                       | 5 to 8     |             |    |
| 0.34 | 0.35                                  | 0.13 | 0.08  | 3.46         | 5 to 7 | 5 to 7                                       | 4 to 7     |             |    |
| 0.47 | 0.80                                  | 0.31 | 0.08  | 3.42         | 4 to 7 | 4 to 6                                       | 4 to 6     |             |    |

Table I—Continued

| Composition of steel (remainder iron) |      |      |      |       |              | Grain No. of case after carburizing 8 hours |            |             |
|---------------------------------------|------|------|------|-------|--------------|---------------------------------------------|------------|-------------|
| 5                                     | % C  | % Mn | % Si | % Cr  | Other metals | At 925° C.                                  | At 975° C. | At 1025° C. |
|                                       | 0.18 | 0.45 | 0.24 | None  | 0.75         | 3 to 7                                      | 1 to 8     | 1 to 3      |
| 10                                    | 0.22 | 0.46 | 0.27 | 0.10  | 0.75         | 7 to 8                                      | 5 to 8     | 5 to 8      |
|                                       | 0.49 | 0.68 | 0.24 | 0.07  | 1.05         | 4 to 6                                      | 4 to 6     | 4 to 7      |
|                                       | 0.28 | 0.53 | 0.36 | 0.08  | 2.94         | 8                                           | 8          | 7 to 7      |
|                                       | 0.46 | 0.78 | 0.78 | 0.11  | 0.51         | 6 to 8                                      | 5 to 8     | 5 to 7      |
|                                       | 0.17 | 0.43 | 0.19 | None  | 0.33         | 2 to 8                                      | 2 to 6     | 1 to 5      |
|                                       | 0.35 | 0.42 | 0.16 | None  | 0.31         | 2 to 5                                      | 1 to 6     | 1 to 3      |
| 15                                    | 0.18 | 0.37 | 0.18 | 0.084 | 0.32         | 6 to 8                                      | 6 to 8     | 6 to 8      |
|                                       | 0.33 | 0.40 | 0.17 | 0.10  | 0.16         | 7 to 9                                      | 9          | 9           |
|                                       | 0.13 | 0.42 | 0.16 | None  | 1.25         | 0.44                                        | 2 to 7     | 2 to 6      |
|                                       | 0.34 | 0.41 | 0.13 | None  | 1.34         | 0.47                                        | 3 to 9     | 3 to 8      |
|                                       | 0.14 | 0.43 | 0.21 | 0.09  | 1.24         | 0.59                                        | 4 to 8     | 5 to 7      |
| 20                                    | 0.39 | 0.43 | 0.12 | 0.07  | 1.27         | 0.61                                        | 4 to 8     | 4 to 8      |
|                                       | 0.47 | 0.60 | 0.14 | 0.11  | 1.61         | 0.68                                        | 4 to 8     | 4 to 6      |
|                                       | 0.17 | 0.41 | 0.31 | None  | 3.40         | 1.25                                        | 3 to 8     | 2 to 6      |
|                                       | 0.32 | 0.38 | 0.18 | None  | 3.57         | 1.49                                        | 4 to 7     | 3 to 7      |
|                                       | 0.14 | 0.36 | 0.16 | 0.08  | 3.45         | 1.46                                        | 6 to 8     | 5 to 8      |
| 25                                    | 0.34 | 0.37 | 0.14 | 0.10  | 3.53         | 1.46                                        | 4 to 6     | 6 to 7      |
|                                       | 0.18 | 0.50 | 0.22 | None  | 1.74         | 0.24                                        | 4 to 7     | 1 to 6      |
|                                       | 0.31 | 0.42 | 0.09 | None  | 1.74         | 0.25                                        | 8          | 2 to 7      |
|                                       | 0.15 | 0.44 | 0.23 | 0.09  | 1.72         | 0.22                                        | 9          | 9           |
|                                       | 0.40 | 0.43 | 0.23 | 0.10  | 1.77         | 0.14                                        | 9          | 8 to 9      |
| 30                                    | 0.20 | 0.80 | 0.24 | None  | 0.58         | 0.21                                        | 3 to 7     | 1 to 6      |
|                                       | 0.35 | 0.68 | 0.15 | None  | 0.96         | 0.25                                        | 3 to 5     | 1 to 6      |
|                                       | 0.15 | 0.67 | 0.20 | 0.09  | 0.63         | 0.22                                        | 7 to 8     | 5 to 8      |
|                                       | 0.37 | 0.71 | 0.27 | 0.10  | 1.00         | 0.17                                        | 4 to 7     | 4 to 7      |
|                                       | 0.51 | 0.64 | 0.23 | 0.10  | 1.03         | 0.10                                        | 5 to 6     | 5 to 7      |

In general, the grain refining effect is roughly proportional to the columbium content up to a certain optimum amount of columbium, which optimum content depends chiefly on the carbon content of the steel. The grain refinement of a maximum 0.1% carbon steel reaches substantially its greatest degree at about 0.1% columbium; a 0.15% carbon steel at about 0.15% columbium; a 0.35% carbon steel at about 0.18% columbium; and a 0.5% carbon steel at about 0.25% columbium. The presence of chromium, molybdenum, or vanadium reduces somewhat these optimum amounts of columbium. A moderate excess of columbium above the optimum and below the maximum specified above (1%), will not ordinarily adversely affect the properties of the steel to a serious extent.

The influence of columbium on the tensile and impact properties of the steels under consideration is indicated by the data appearing in Tables II and III which show the experimentally determined yield point in thousands of pounds per

square inch (Y. P.), maximum stress in thousands of pounds per square inch (M. S.), percentage elongation in a 2 inch gage length (El. %), and reduction in area (R. A. %), all on 0.505 inch diameter A. S. T. M. standard tensile test pieces; and also the Izod impact value in foot pounds as determined on a standard Izod machine with an initial energy level of 120 foot pounds and a standard specimen one centimeter square provided with a 45° notch.

Table II

| Composition of steel (remainder iron)                       |            |            |            |            |            | Y. P. 1000 | M. S. 1000 | El. per cent | R. A. per cent | Izod ft.-lb. |
|-------------------------------------------------------------|------------|------------|------------|------------|------------|------------|------------|--------------|----------------|--------------|
| Percent C                                                   | Percent Mn | Percent Si | Percent Cr | Percent Ni | Percent Mo | lb/sq. in. | lb/sq. in. |              |                |              |
| <i>As-rolled</i>                                            |            |            |            |            |            |            |            |              |                |              |
| 0.09                                                        | 0.30       | 0.20       | None       | 48         | 57.5       | 35         | 63         | 76           |                |              |
| 0.08                                                        | 0.25       | 0.20       | 0.28       | 60.5       | 65         | 26         | 69         | 93           |                |              |
| 0.10                                                        | 0.33       | 0.42       | 0.65       | 24         | 58.5       | 40         | 80         | 98           |                |              |
| <i>Air cooled from 900° C.</i>                              |            |            |            |            |            |            |            |              |                |              |
| 0.09                                                        | 0.30       | 0.20       | None       | 41         | 55         | 39         | 64         | 82           |                |              |
| 0.08                                                        | 0.25       | 0.20       | 0.28       | 55         | 60.5       | 27         | 68         | 95           |                |              |
| 0.10                                                        | 0.33       | 0.42       | 0.65       | 22.3       | 57.6       | 40         | 81         | 92           |                |              |
| <i>Quenched in water from 900° C.; and drawn at 150° C.</i> |            |            |            |            |            |            |            |              |                |              |
| 0.16                                                        | 0.46       | 0.20       | None       | 64.5       | 100        | 17         | 55         | 42           |                |              |
| 0.15                                                        | 0.45       | 0.27       | 0.017      | 72.5       | 89         | 27         | 63         | 75           |                |              |
| 0.17                                                        | 0.48       | 0.28       | 0.45       | 71         | 81.8       | 31         | 71         | 75           |                |              |
| <i>Air cooled from 925° C.</i>                              |            |            |            |            |            |            |            |              |                |              |
| 0.16                                                        | 0.46       | 0.29       | None       | 46.5       | 66.8       | 33         | 55         | 72           |                |              |
| 0.15                                                        | 0.45       | 0.27       | 0.017      | 50         | 67.5       | 33         | 62         | 72           |                |              |
| 0.17                                                        | 0.48       | 0.28       | 0.45       | 50         | 63.5       | 36         | 69         | 75           |                |              |
| <i>Quenched in water from 850° C.; and drawn at 550° C.</i> |            |            |            |            |            |            |            |              |                |              |
| 0.41                                                        | 0.77       | 0.27       | None       | 101.5      | 125.5      | 19         | 51         | 37           |                |              |
| 0.38                                                        | 0.80       | 0.27       | 0.06       | 91.5       | 110.5      | 21         | 57         | 47           |                |              |
| 0.43                                                        | 0.74       | 0.22       | 0.36       | 87         | 105        | 24         | 55         | 49           |                |              |
| <i>Cooled in air from 875° C.</i>                           |            |            |            |            |            |            |            |              |                |              |
| 0.41                                                        | 0.77       | 0.27       | None       | 62         | 91         | 25         | 48         | 15           |                |              |
| 0.38                                                        | 0.80       | 0.27       | 0.06       | 65         | 90.5       | 21         | 57         | 28           |                |              |
| 0.43                                                        | 0.74       | 0.22       | 0.36       | 64.5       | 86         | 24         | 56         | 40           |                |              |

Table III

| Composition of steel (remainder iron)                                       |            |            |            |            |            |            | Y. P. | M. S. | El. per cent | R. A. percent | Izod ft.-lb. |
|-----------------------------------------------------------------------------|------------|------------|------------|------------|------------|------------|-------|-------|--------------|---------------|--------------|
| Percent C                                                                   | Percent Mn | Percent Si | Percent Cr | Percent Ni | Percent Mo | Percent Cb |       |       |              |               |              |
| <i>Quenched in oil from 850° C.-900° C.; drawn in air at 150° C.-45° C.</i> |            |            |            |            |            |            |       |       |              |               |              |
| 0.18                                                                        | 0.45       | 0.24       | 0.75       | —          | —          | 0.10       | 61    | 97    | 22           | 50            | 33           |
| 0.22                                                                        | 0.46       | 0.27       | 0.75       | —          | —          | —          | 72    | 116   | 19           | 49            | 34           |
| 0.35                                                                        | 0.43       | 0.25       | 2          | —          | —          | —          | 191   | 204   | 9            | 37            | 7            |
| 0.32                                                                        | 0.33       | 0.18       | 1.83       | —          | —          | 0.11       | 193   | 218   | 9            | 37            | 11           |
| 0.41                                                                        | 0.40       | 0.28       | 2          | —          | —          | 0.43       | 197   | 217   | 9            | 37            | 9            |
| 0.13                                                                        | 0.42       | 0.16       | 0.44       | 1.25       | —          | —          | 71    | 100   | 24           | 60            | 57           |
| 0.18                                                                        | 0.43       | 0.21       | 0.59       | 1.24       | —          | 0.09       | 68    | 108   | 20           | 66            | 46           |
| 0.44                                                                        | 0.75       | 0.25       | 0.65       | 1.5        | —          | —          | 181   | 204   | 10           | 35            | 9            |
| 0.49                                                                        | 0.75       | 0.25       | 0.65       | 1.5        | —          | 0.42       | 177   | 194   | 12           | 44            | 10           |
| 0.17                                                                        | 0.43       | 0.19       | —          | —          | 0.33       | —          | 58    | 88    | 26           | 68            | 74           |
| 0.17                                                                        | 0.45       | 0.25       | —          | —          | 0.35       | 0.17       | 47    | 72    | 35           | 67            | 81           |
| 0.18                                                                        | 0.50       | 0.22       | —          | 1.74       | 0.24       | —          | 81    | 117   | 18           | 43            | 34           |
| 0.16                                                                        | 0.45       | 0.25       | —          | 1.75       | 0.28       | 0.18       | 55    | 94    | 26           | 69            | 77           |
| 0.20                                                                        | 0.80       | 0.24       | 0.58       | —          | 0.21       | —          | 99    | 125   | 13           | 38            | 21           |
| 0.18                                                                        | 0.75       | 0.25       | 0.6        | —          | 0.25       | 0.23       | 77    | 119   | 21           | 45            | 49           |

Table III—Continued

| 5                                  | Composition of steel (remainder iron) |               |               |               |               |               |               | Y. P. | M. S. | El.<br>per-<br>cent | R. A.<br>percent | Izod<br>ft.-lb. | 5  |    |
|------------------------------------|---------------------------------------|---------------|---------------|---------------|---------------|---------------|---------------|-------|-------|---------------------|------------------|-----------------|----|----|
|                                    | Percent<br>C                          | Percent<br>Mn | Percent<br>Si | Percent<br>Cr | Percent<br>Ni | Percent<br>Mo | Percent<br>Cb |       |       |                     |                  |                 |    |    |
| Cooled in air from 850° C.—900° C. |                                       |               |               |               |               |               |               |       |       |                     |                  |                 |    |    |
| 10                                 | 0.18                                  | 0.45          | 0.24          | 0.75          |               |               |               | 59    | 72    | 35                  | 67               | 72              | 10 |    |
|                                    | 0.22                                  | 0.46          | 0.27          | 0.75          |               |               |               | 59    | 76    | 34                  | 69               | 79              |    |    |
|                                    | 0.35                                  | 0.43          | 0.25          | 2             |               |               |               | 102   | 149   | 11                  | 23               | 5               |    |    |
|                                    | 0.32                                  | 0.33          | 0.15          | 1.83          |               |               |               | 0.11  | 71    | 113                 | 20               | 59              | 33 |    |
|                                    | 0.41                                  | 0.40          | 0.25          | 2             |               |               |               | 0.43  | 136   | 191                 | 10               | 18              | 6  |    |
|                                    | 0.13                                  | 0.42          | 0.16          | 0.44          | 1.25          |               |               | 47    | 69    | 34                  | 66               | 75              |    |    |
|                                    | 0.14                                  | 0.43          | 0.21          | 0.59          | 1.24          |               |               | 0.09  | 60    | 73                  | 30               | 54              | 79 |    |
|                                    | 0.44                                  | 0.75          | 0.25          | 0.65          | 1.5           |               |               | 105   | 148   | 12                  | 32               | 4               |    |    |
| 15                                 | 0.49                                  | 0.75          | 0.25          | 0.65          | 1.5           |               |               | 0.42  | 121   | 161                 | 9                | 18              | 7  | 15 |
|                                    | 0.17                                  | 0.43          | 0.19          |               |               |               |               | 0.33  | 52    | 70                  | 34               | 61              | 72 |    |
|                                    | 0.17                                  | 0.45          | 0.25          |               |               |               |               | 0.35  | 55    | 87                  | 31               | 70              | 80 |    |
|                                    | 0.18                                  | 0.50          | 0.22          |               |               |               |               | 0.17  | 52    | 87                  | 27               | 52              | 49 |    |
|                                    | 0.16                                  | 0.45          | 0.25          |               |               |               |               | 1.74  | 0.24  | 57                  | 77               | 35              | 69 | 52 |
|                                    | 0.20                                  | 0.80          | 0.24          | 0.58          |               |               |               | 1.75  | 0.25  | 0.18                | 53               | 90              | 24 | 48 |
|                                    | 0.18                                  | 0.75          | 0.25          | 0.6           |               |               |               | 0.21  | 44    | 82                  | 31               | 63              | 73 |    |

20 It will be observed from the data of Tables II and III that, in the steels containing up to about 0.3% carbon, the addition of up to about 0.1% columbium increases the yield point, maximum stress, and ratio of yield point to maximum stress.

25 The ductility is only slightly affected. As the columbium is increased above 0.1%, the softening effect of the columbium begins to predominate, the yield point and maximum stress are decreased,

30 and the ductility is substantially increased. As the carbon content is increased above 0.3%, and as other alloyed additions are made, the effects of columbium on the tensile properties are reduced, particularly if the steels are heat treated.

35 It will also be noted in Tables II and III that the addition of columbium raises the impact strength of the steels, and that the improvement is greatest in the high carbon steels and those containing chromium.

40 As mentioned above, the addition of columbium to the plain carbon and low alloyed steels considerably increases their impact strength at sub-zero temperatures. As little as 0.2% columbium raises the impact strength at -100° C. to 10 foot pounds or more.

45 Table IV contains impact data obtained in the manner described in connection with Tables II and III, except that the samples under the heading "-78° C." were cooled about an hour at -78° C. in a bath of acetone and frozen carbon dioxide before testing; and the samples under the heading "-100° C." were cooled about an hour at -100° C. in liquid propane which in turn was cooled with liquid air, before testing. After cooling, the specimens were rapidly transferred from the cooling medium to the Izod machine and tested. The time required for the transfer and test was in all cases less than ten seconds.

Table IV

| 60 | Composition of steel (remainder iron) |               |               |               |              | Izod impact ft.-lbs., at— |         |          | 60   |  |
|----|---------------------------------------|---------------|---------------|---------------|--------------|---------------------------|---------|----------|------|--|
|    | Percent<br>C                          | Percent<br>Mn | Percent<br>Si | Percent<br>Cb | Other metals | +28° C.                   | -78° C. | -100° C. |      |  |
| 65 | 0.21                                  | 0.4           | 0.3           | None          |              | None                      | 56      | 4        | 2    |  |
|    | 0.18                                  | 0.5           | 0.3           | 0.08          |              | None                      | 58      | 16.5     | 5    |  |
|    | 0.20                                  | 0.5           | 0.3           | 0.20          |              | None                      | 67      | 30       | 10   |  |
|    | 0.24                                  | 0.7           | 0.4           | 0.32          |              | None                      | 67      | 34.5     | 15   |  |
|    | 0.20                                  | 0.6           | 0.3           | 0.67          |              | None                      | 74      | 37       | 21.5 |  |
|    | 0.23                                  | 0.6           | 0.4           | 0.73          |              | None                      | 84      | 75       | 40   |  |
|    | 0.17                                  | 1.6           | 0.3           | 0.12          |              | None                      | 86      | 50       |      |  |
|    | 0.17                                  | 0.5           | 0.3           | 0.10          |              | 3.5% Ni                   | 73      | 50       |      |  |
|    | 0.22                                  | 0.5           | 0.3           | 0.10          |              | 0.75% Cr                  | 79      | 37       |      |  |
|    | 0.16                                  | 0.4           | 0.2           | 0.10          |              | 1% Cr, 0.2% V             | 83      | 69       |      |  |
|    | 0.14                                  | 0.4           | 0.2           | 0.09          |              | 0.6% Cr, 1.2% Ni          | 79      | 69       |      |  |
|    | 0.15                                  | 0.4           | 0.2           | 0.09          |              | 0.22% Mo, 1.7% Ni         | 68      | 70       |      |  |
| 70 | 0.18                                  | 0.8           | 0.3           | 0.46          |              | 0.8% Cr, 1.05% Cu         | 82      | 86       | 82   |  |

20 The presence of columbium substantially increases the resistance of these steels to hot oxidation and, although the columbium steels are not to be considered oxidation resistant in the sense that high chromium steels, for instance, are oxidation resistant, the increase in resistance will be valuable in many uses of the steels. Table V presents data illustrating this effect of columbium.

Table V

| Composition of steel (remainder iron) |               |               |               | Percent loss in weight after 1,176 hours at 650° C. |
|---------------------------------------|---------------|---------------|---------------|-----------------------------------------------------|
| Percent<br>C                          | Percent<br>Mn | Percent<br>Si | Percent<br>Cb |                                                     |
| 0.09                                  | 0.30          | 0.20          | None          | 10                                                  |
| 0.09                                  | 0.15          | 0.74          | None          | 5.7                                                 |
| 0.06                                  | 0.41          | 0.28          | 0.41          | 4.4                                                 |
| 0.07                                  | 0.41          | 0.41          | 0.94          | 2.8                                                 |

30 The invention is based on the above-described discoveries and comprises new alloy steels and articles composed thereof, having in addition to 0.02% to 1% columbium, substantially the limits of composition indicated in Table VI.

Table VI

| Type of steel | Composition limits (remainder iron) |            |            |                               | 50 |
|---------------|-------------------------------------|------------|------------|-------------------------------|----|
|               | Percent C                           | Percent Mn | Percent Si | Other metals                  |    |
| C.....        | Up to 1...                          | Up to 2... | Up to 1... | None                          |    |
| Cr.....       | Up to 0.6                           | Up to 2    | Up to 1    | 0.25 to 2% Cr.                |    |
| Cr-Ni.....    | Up to 0.6                           | Up to 1    | Up to 1    | 0.05 to 5% Ni, 0.25 to 2% Cr. |    |
| Mo.....       | Up to 0.6                           | Up to 2    | Up to 1    | 0.05 to 1% Mo.                |    |
| Mo-Ni.....    | Up to 0.6                           | Up to 1    | Up to 1    | 0.05 to 5% Ni, 0.05 to 1% Mo. | 55 |
| Cr-Mo.....    | Up to 0.6                           | Up to 2    | Up to 1    | 0.25 to 2% Cr, 0.05 to 1% Mo. |    |

| 65   | Composition of steel (remainder iron) |               |               |               |                   | 60   |
|------|---------------------------------------|---------------|---------------|---------------|-------------------|------|
|      | Percent<br>C                          | Percent<br>Mn | Percent<br>Si | Percent<br>Cb | Other metals      |      |
| 0.21 | 0.4                                   | 0.3           | None          |               | None              | 2    |
| 0.18 | 0.5                                   | 0.3           | 0.08          |               | None              | 5    |
| 0.20 | 0.5                                   | 0.3           | 0.20          |               | None              | 10   |
| 0.24 | 0.7                                   | 0.4           | 0.32          |               | None              | 15   |
| 0.20 | 0.6                                   | 0.3           | 0.67          |               | None              | 21.5 |
| 0.23 | 0.6                                   | 0.4           | 0.73          |               | None              | 40   |
| 0.17 | 1.6                                   | 0.3           | 0.12          |               | None              |      |
| 0.17 | 0.5                                   | 0.3           | 0.10          |               | 3.5% Ni           |      |
| 0.22 | 0.5                                   | 0.3           | 0.10          |               | 0.75% Cr          |      |
| 0.16 | 0.4                                   | 0.2           | 0.10          |               | 1% Cr, 0.2% V     |      |
| 0.14 | 0.4                                   | 0.2           | 0.09          |               | 0.6% Cr, 1.2% Ni  |      |
| 0.15 | 0.4                                   | 0.2           | 0.09          |               | 0.22% Mo, 1.7% Ni |      |
| 0.18 | 0.8                                   | 0.3           | 0.46          |               | 0.8% Cr, 1.05% Cu |      |

65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930

The articles of the invention include articles deep-drawn from the steel of the invention; articles having a core containing less than 0.5% carbon and a carburized case containing more than 0.8% carbon, and 0.02% to 1% columbium throughout, the remainder of the composition being as shown in Table VI; parts of machines and of other apparatus, required to withstand stress at moderately elevated temperatures; articles, composed of the steel of the invention, designed for use to resist impact shock at subzero temperatures; and pressure vessels, composed of the steel of the invention, designed to withstand two or three dimensional stress at subzero temperatures.

It will be appreciated that the specific examples herein are given by way of illustration, and that the invention is not limited to or by such examples.

We claim:

20. 1. Low alloyed steel containing carbon in an amount not exceeding 0.6%; manganese in an amount not exceeding 2%; silicon in an amount not exceeding 1%; a substantial amount of at least one carbide forming metal of the group consisting of chromium and molybdenum, the chromium being less than 2% and the molybdenum not exceeding 1%; 0.02% to 0.5% columbium which imparts to said steel a fine-grained structure which persists at all temperatures up to and somewhat above the critical range, increased ductility, increased impact strength at normal and subzero temperatures, improved hot and cold workability, and increased resistance to hot and cold oxidation, but does not impart substantial age hardening properties; and the remainder iron.
25. 2. Steel containing carbon in an amount not exceeding 0.6%, manganese in an amount not exceeding 2%, silicon in an amount not exceeding 1%, 0.25% to less than 2% chromium, 0.02% to 0.5% columbium which imparts to said steel a fine-grained structure which persists at all temperatures up to and somewhat above the critical range, increased ductility, increased impact strength at normal and subzero temperatures, improved hot and cold workability, and increased resistance to hot and cold oxidation, but does not impart substantial age hardening properties, the remainder iron.
30. 3. Steel containing carbon in an amount not exceeding 0.6%, manganese in an amount not exceeding 2%, silicon in an amount not exceeding 1%, 0.25% to less than 2% chromium, 0.02% to 0.5% columbium which imparts to said steel a fine-grained structure which persists at all temperatures up to and somewhat above the critical range, increased ductility, increased impact strength at normal and subzero temperatures, improved hot and cold workability, and increased resistance to hot and cold oxidation, but does not impart substantial age hardening properties, the remainder iron.
35. 4. Steel containing carbon in an amount not exceeding 0.6%, manganese in an amount not exceeding 2%, silicon in an amount not exceeding 1%, 0.25% to less than 2% chromium, 0.02% to 0.5% columbium which imparts to said steel a fine-grained structure which persists at all temperatures up to and somewhat above the critical range, increased ductility, increased impact strength at normal and subzero temperatures, improved hot and cold workability, and increased resistance to hot and cold oxidation, but does not impart substantial age hardening properties, the remainder iron.
40. 5. Steel containing carbon in an amount not exceeding 0.6%, manganese in an amount not exceeding 2%, silicon in an amount not exceeding 1%, 0.25% to less than 2% chromium, 0.02% to 0.5% columbium which imparts to said steel a fine-grained structure which persists at all temperatures up to and somewhat above the critical range, increased ductility, increased impact strength at normal and subzero temperatures, improved hot and cold workability, and increased resistance to hot and cold oxidation, but does not impart substantial age hardening properties, the remainder iron.
45. 6. Steel containing carbon in an amount not exceeding 0.6%, manganese in an amount not exceeding 2%, silicon in an amount not exceeding 1%, 0.25% to less than 2% chromium, 0.02% to 0.5% columbium which imparts to said steel a fine-grained structure which persists at all temperatures up to and somewhat above the critical range, increased ductility, increased impact strength at normal and subzero temperatures, improved hot and cold workability, and increased resistance to hot and cold oxidation, but does not impart substantial age hardening properties, the remainder iron.
50. 7. Machine element subject to impact stress at elevated temperatures below 500° C. and composed of a low alloyed steel containing carbon in an amount not exceeding 0.6%; manganese in an amount not exceeding 2%; silicon in an amount not exceeding 1%; a substantial amount of at least one carbide forming metal of the group consisting of chromium and molybdenum, the chromium being less than 2% and the molybdenum not exceeding 1%; 0.02% to 0.5% columbium which imparts to said element a persistent fine-grained structure, increased ductility, and increased impact strength at working temperatures, remainder iron.

ing 1%, 0.05% to 1% molybdenum, 0.02% to 0.5% columbium, the remainder iron.

4. Steel containing carbon in an amount not exceeding 0.6%, manganese in an amount not exceeding 2%, silicon in an amount not over 5 1%, 0.05% to 1% molybdenum, 0.25% to less than 2% chromium, 0.02% to 0.5% columbium, the remainder iron.

5. Case carburized article having a core containing less than 0.5% carbon and a carburized 10 case containing more than 0.8% carbon, the core and case being composed of steel containing, aside from carbon, manganese in an amount not exceeding 2%; silicon in an amount not exceeding 1%; a substantial amount of at least one 15 carbide forming metal of the group consisting of chromium and molybdenum, the chromium being less than 2% and the molybdenum not exceeding 1%; 0.02% to 0.5% columbium which imparts to said carburized article a fine-grained structure, increased ductility, and increased impact strength at normal and subzero temperatures; and the remainder iron.

6. Article used to resist, at subzero temperatures, impact shock or multidimensional stress, 25 which article is composed of a low alloyed steel containing carbon in an amount not exceeding 0.6%; manganese in an amount not exceeding 2%; silicon in an amount not exceeding 1%; a substantial amount of at least one carbide forming 30 metal of the group consisting of chromium and molybdenum, the chromium being less than 2% and the molybdenum not exceeding 1%; 0.02% to 0.5% columbium which imparts to said article increased impact strength at subzero temperatures; and the remainder iron.

7. Machine element subject to impact stress at elevated temperatures below 500° C. and composed of a low alloyed steel containing carbon in an amount not exceeding 0.6%; manganese in an amount not exceeding 2%; silicon in an amount not exceeding 1%; a substantial amount of at least one carbide forming metal of the group consisting of chromium and molybdenum, the chromium being less than 2% and the molybdenum not exceeding 1%; 0.02% to 0.5% columbium which imparts to said element a persistent fine-grained structure, increased ductility, and increased impact strength at working temperatures, remainder iron.

FREDERICK M. BECKET.  
RUSSELL FRANKS.